

Nov. 29, 1955

H. C. YUTZY ET AL

2,725,298

TRANSFER PROCESS OF PHOTOGRAPHIC PRINTING

Filed May 3, 1952

**Fig. 1**



**Fig. 2**



**Henry C. Yutzy  
Herbert B. Cowden**  
INVENTORS

BY *Daniel J. Mayne,  
R. Frank Smith*

ATTORNEYS

1

2,725,298

TRANSFER PROCESS OF PHOTOGRAPHIC  
PRINTING

Henry C. Yutzy and Herbert B. Cowden, Rochester, N. Y.,  
assignors to Eastman Kodak Company, Rochester,  
N. Y., a corporation of New Jersey

Application May 3, 1952, Serial No. 285,855

3 Claims. (Cl. 95—88)

This invention relates to photography and particularly to a transfer process of printing a photographic image.

Various methods of forming an image in an unsensitized sheet by transfer from an originally sensitive layer have been described in the literature. In application Serial No. 783,913, filed November 4, 1947, now Patent No. 2,596,754, E. C. Yackel has described a procedure according to which a photographic image formed in an unhardened gelatin layer by conventional processing is transferred to a dry absorbent receiving sheet by squeegeeing the print, after processing, into contact with the dry absorbent surface, then stripping the two apart after a short interval of contact. In this process a stratum of the gelatin layer is adhered to the receiving surface and transferred leaving behind the remainder of the gelatin layer containing part of the image. Upon rewetting the gelatin layer successive transfers can be made. This method produces a negative transferred image if a positive is used to make the original exposure.

Processes involving solvent transfer methods have also been described in the literature, a review of these appearing in an article by Varden in the Photographic Society of America Journal, vol. 13, September 1947, page 551. These processes involve development of an exposed silver halide emulsion layer with a developing solution containing a solvent for silver halide. During or immediately following initial development the exposed emulsion layer is placed in contact with another layer, usually unsensitized, and the dissolved silver salts representing the positive image are then transported to the second layer and deposited as a positive image. This method gives a positive transferred image if a positive image is used for the original exposure.

We have now found that an image formed in the outer of two superposed strata by the solvent transfer method may be transferred to the receiving sheet by the method of Patent 2,596,754 and that several successive transfers may be made in this way to produce duplicate images. Our method involves in general the use as the sensitive material of a photographic element comprising a support having a silver halide emulsion layer thereon and an unhardened colloid layer overcoated on the emulsion layer so that the colloid layer is outermost. The colloid layer has dispersed therein an agent for promoting image formation, comprising physical development nuclei or a chemical precipitant for dissolved silver ions, so that the dissolved silver salts transported to the colloid layer from the silver halide emulsion layer during solvent development, are deposited and retained in a visible form in the colloid layer. The image thus obtained in the colloid layer may be transferred layer-wise to an absorbent support and successive transfers of the colloid layer containing the image may be made on successive absorbent supports to produce duplicate images.

In the drawing, Fig. 1 illustrates sectional views of the photographic elements at various stages in our preferred process, and

2

Fig. 2 is a sectional view of a modified form of the sensitive element used according to our invention.

The silver halide emulsion used in the sensitive element of our invention may be an ordinary unsensitized gelatinous silver halide emulsion, or an optically sensitized or chemically sensitized emulsion, in which the gelatin is substantially unhardened or hardened in such a way that it does not harden the colloid layer coated over it, as explained more fully hereinafter. The emulsion may contain a substantially non-diffusing developing agent of the tanning type as disclosed in Yackel application Serial No. 783,912, filed November 4, 1947, now Patent No. 2,592,368 or a non-tanning, substantially non-diffusing developing agent as described in application Serial No. 267,447, filed January 21, 1952, by Yutzy and Yackel.

The colloid layer coated over the emulsion layer is a layer of water-susceptible or water-permeable colloid, such as gelatin or polyvinyl alcohol, containing an agent promoting image formation and capable of yielding with silver ion a dark-color silver substance, when the dissolved silver salts from the emulsion layer come in contact with it. This agent in the colloid layer may comprise either physical development nuclei or a chemical precipitant for dissolved silver ions, the following being suitable agents:

Colloidal silver  
Colloidal sulphur  
Stannous chloride  
Sodium stannite  
30 Sodium sulfide  
Zinc sulfide  
Cadmium sulfide  
Arsenous oxide  
35 Aminoguanidine sulfate  
Aminoguanidine carbonate  
Organic sulfiding agents, e. g.  
Mercaptates  
Xanthates  
40 Thioacetates  
Thiourea or its derivatives  
Substituted hydrazines

The developing solution may be the usual and customary type of photographic developing solution containing hydroquinone, N-methyl-p-aminophenol sulfate, p-phenylene diamine, etc., or any mixture of these, as the developing agent and containing the usual ingredients such as alkali, potassium bromide and sodium sulfite. If the developing agent is incorporated in the emulsion layer 45 the solution used to effect development may be a simple alkaline solution such as a sodium carbonate or sodium hydroxide solution. The developing solution must also contain a silver halide solvent such as sodium thiosulfate, sodium sulfite, ammonium hydroxide, ammonium sulfate, 50 ammonium nitrate, ammonium chloride or a thiocyanate of an alkali metal. If the silver halide solvent is contained in the sensitive element as shown in Examples 3 and 4 hereinafter, the developing solution need not of course contain a silver halide solvent.

If a non-diffusing developing agent is to be used in the sensitive emulsion, any of the following compounds will serve for this purpose:

3,4-dihydroxy-diphenyl  
2,5-dihydroxy-diphenyl  
65 2,3-dihydroxy-diphenyl  
5,6,7,8-tetrahydronaphthol hydraquinone  
2-hydroxy-5-amino-diphenyl  
3,4-diamino-diphenyl  
Dodecyl catechol  
70 Diamyl-hydroquinone  
Lauryl hydroquinone

Our invention will be further illustrated by reference to the following specific examples.

*Example 1*

An ordinary photographic paper stock free from formaldehyde or other compound capable of hardening gelatin was coated with a high contrast contact speed gelatino-silver chloride emulsion substantially free of gelatin hardeners. On this photographic emulsion layer there was coated a layer of substantially unhardened gelatin containing colloidal zinc sulfide. This suspension was prepared as follows:

A

157 cc. H<sub>2</sub>O  
23 cc. Fused Na<sub>2</sub>S—1 g. in 1000 cc. H<sub>2</sub>O

B

100 cc. Zn(NO<sub>3</sub>)<sub>2</sub>·6H<sub>2</sub>O—1 g. in 1000 cc. H<sub>2</sub>O

B was poured into A at room temperature with rapid stirring. The mixture was quickly poured into 110 g. 20 percent gelatin (containing 10 cc. 7.5 percent aqueous saponin) at 40° C. The whole was held at 40° C. for coating.

This composite element was exposed to a positive original and the silver halide emulsion layer developed to a negative in a developing solution of the following composition:

|                                                                  |     |
|------------------------------------------------------------------|-----|
| N-methyl-p-aminophenol sulfate                                   | 10  |
| Hydroquinone                                                     | 10  |
| Sodium sulfite, desiccated                                       | 50  |
| Sodium metaborate                                                | 15  |
| NaOH                                                             | 15  |
| KBr                                                              | 0.5 |
| Na <sub>2</sub> S <sub>2</sub> O <sub>3</sub> ·5H <sub>2</sub> O | 5   |
| Urea                                                             | 20  |
| Chlorobenzotriazole                                              | 0.5 |
| Water to 1 liter                                                 |     |

After development for approximately one minute there was formed in the nucleating layer a positive image. The sheet was removed from the developer solution, squeegeed to remove excess developer and pressed into contact with a sheet of absorbent paper, for example an ordinary bond typewriter paper. After a few seconds the photographic sheet was stripped from the receiving paper, which was found to carry a positive image representing a stratum of the total positive image formed in the over-coated nucleating layer.

The original photographic layer carrying the negative and the remainder of the nucleating layer with the positive image was rewet in the developer solution, squeegeed and rolled into contact with a second sheet of receiving paper, then stripped as before leaving another portion of the image on the second receiving sheet. This operation could be repeated several times.

The incorporation of from 1 to 20 per cent of urea in the developing bath to increase the softness of the gelatin image was found to be advantageous.

*Example 2*

An ordinary photographic paper stock was coated with a high contrast contact speed gelatino-silver chloride emulsion hardened with 4.9 cc. of 20 per cent formaldehyde solution per kilogram of emulsion. On this emulsion layer there was coated a layer of polyvinyl alcohol containing cadmium sulfide prepared as follows:

A. 46 grams of a 17% solution of polyvinyl alcohol in water (which is a gel) was mixed with 234 cc. of water and melted at 80° C. The solution was cooled to 40° C. and mixed with 14.4 cc. of a Na<sub>2</sub>S solution which had been made by dissolving 1 gram of fused Na<sub>2</sub>S in sufficient water to make 100 cc. of solution.

B. 45.6 cc. of CdCl<sub>2</sub>·2½H<sub>2</sub>O solution which had been made by dissolving 1 gram of the cadmium chloride in sufficient water to make 100 cc. of solution was prepared at room temperature.

5 5 B added to A with rapid stirring. Finally 10 cc. 7.5% aqueous saponin added. Dispersion held at 40° C. for coating. This composite element after exposure to a positive image and development in the developer of Example 1 was squeegeed to remove excess developer and rolled into contact with an absorbent receiving sheet. The positive image formed in the polyvinyl alcohol layer was transferred to the receiving support, yielding a direct positive image.

10 15 The advantage of this element is that conventional photographic emulsions with conventional hardening agents such as formaldehyde may be used. Such gelatin hardeners have little hardening action on polyvinyl alcohol so that the polyvinyl alcohol layer retains the proper physical characteristics for a transfer to the receiving sheet.

*Example 3*

A photographic paper support free from formaldehyde or other gelatin hardeners bearing instead of the usual baryta coat a similar layer made with barium sulfite instead of barium sulfate was coated with the emulsion layer of Example 1 containing 12 g. of 3,4-dihydroxy diphenyl per kilogram of emulsion and also the nucleating layer of Example 1. The nucleating layer could 20 25 also be coated on a separate sheet and squeegeed into contact with the emulsion layer just prior to the development process. The barium sulfite layer was made as follows:

|                                     |                            |
|-------------------------------------|----------------------------|
| G. 30                               | A                          |
| H <sub>2</sub> O (65° C.)           | 750 cc.                    |
| BaCl <sub>2</sub> ·H <sub>2</sub> O | 213 g.                     |
|                                     | B                          |
| 40                                  | H <sub>2</sub> O (boiling) |

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 894

It is also desirable in this case to add some neutral sulfate such as sodium sulfate to the developer since barium sulfate is considerably less soluble than the carbonate, hydroxide or sulfite and will effect a more nearly complete conversion of the barium sulfite to sulfate, thus liberating the soluble sulfite more efficiently.

Other solvent systems may be substituted for the barium sulfite such as calcium or strontium sulfite. Other examples of solvents are slightly soluble or non-wandering ammonium salts or amines. Long-chain amines may be included in the undercoat by coating high molecular resins in the layer as complexes with the amines, the complexes being broken up by the action of the alkali in the developer.

A separate receiving sheet bearing the nucleating layer 15 may be used in conjunction with a conventional silver halide paper, by incorporating the insoluble or non-wandering solvent in the nucleating layer or under the nucleating layer on the receiving sheet. It will be apparent also that the silver halide emulsion may contain a substantially non-diffusing developing agent as described in Example 3, the chemical energy required for formation of the positive image being obtained from suitable reagents in a second layer either overcoated on the emulsion layer or coated on a second transfer sheet.

In the process of Example 1 in which both emulsion and nucleating layer were unhardened it has been found that there is some tendency for the fracture to occur at the paper base during transfer to the receiving sheet, resulting in unwanted transfer of all of the layers. This can be prevented by incorporating in the baryta layer or in a layer beneath the sensitive emulsion layer a completely exposed silver halide emulsion having therein an insoluble tanning developing agent. During development the completely exposed or fogged bottom layer is rapidly developed and tanned at the same time thus hardening the bottom layer and causing it to adhere more strongly to the paper support. This layer may contain the usual baryta or it may contain barium sulfite as described in Example 3. The black density developed in the barium sulfite layer does not affect the transfer results. The following example illustrates a coating made in this way.

#### Example 4

A paper support was coated with a suspension of barium sulfite, silver chloride emulsion, and 4-phenyl catechol as a tanning developing agent. This layer was thoroughly flashed to white light before subsequent coating. Over this layer there was coated a gelatino-silver chloride emulsion also containing 4-phenyl catechol. Over the emulsion there was coated a gelatin layer containing zinc sulfide.

After exposure to an image this material was developed for two to three minutes in an alkaline solution. This caused (1) complete development of the silver in the bottom layer accompanied by tanning of the gelatin in the layer, (2) development of the negative image in the photosensitive layer and solution of the undeveloped silver halide in this layer by the sulfite ion from the bottom layer and (3) diffusion of the silver sulfite complex to the top layer where the silver was deposited as silver sulfide in the form of a positive image. When successive fractions of the top layer were transferred to a receiving support there was little if any tendency for all of the layers to transfer at once.

Our invention will now be described by reference to the accompanying drawing. As shown in Fig. 1 a support 10 has coated thereon a silver halide emulsion layer 11 having exposed portions 12 and unexposed portions 13, an unhardened colloid layer 14 containing a nucleating agent which is coated over the emulsion layer 11. Upon solvent development of this material a silver image 15 is formed in layer 11 and a silver or silver compound image 16 is formed in the nucleating layer by solvent transfer. When this element is rolled into contact with

a receiving sheet 17 a portion 18 of the nucleating layer carrying the image is transferred to the sheet 17 as shown in the final stage of Fig. 1.

Fig. 2 illustrates the modification of our material in 5 which a support 20 is coated with a layer 21 containing an insoluble sulfite, an emulsion layer 22 and a nucleating layer 23.

Where we refer to a "substantially unhardened" gelatin emulsion layer we mean a layer that is not harder than would be the case with gelatin containing 0.25 ounce of formaldehyde (40 per cent, diluted 1 to 3 with water) per pound of gelatin when freshly coated, or 0.1 ounce of the formaldehyde solution per pound of gelatin for a sample aged 3 to 6 months.

Where we refer to "transferring a continuous stratum of the emulsion layer" we mean that a thin layer of the total surface area of the photographic element is carried off onto the receiving support.

It will be understood that the modifications and equivalents included herein are by way of example only and that our invention is to be taken as limited only by the scope of the appended claims.

We claim:

1. The method of photographic reproduction which 25 comprises exposing to a subject a photographic element comprising a support having thereon a silver halide emulsion layer and an unhardened colloid layer on said emulsion layer, said colloid layer having dispersed therein an agent for promoting image formation, selected from the 30 class consisting of physical development nuclei and chemical precipitants for dissolved silver ions, developing said exposed emulsion layer with a silver halide developing agent in the presence of a silver halide solvent to form a negative image in said emulsion layer and a positive image in said colloid layer, and transferring a continuous stratum of said colloid layer to an absorbent support.

2. The method of photographic reproduction which 40 comprises exposing to a subject a photographic element comprising a support having thereon a silver halide emulsion layer and an unhardened gelatin layer on said emulsion layer, said gelatin layer having dispersed therein an agent for promoting image formation, selected from the class consisting of physical development nuclei and chemical precipitants for dissolved silver ions, developing said exposed emulsion layer with a silver halide developing agent in the presence of a silver halide solvent to form a negative image in said emulsion layer and a positive image in said gelatin layer, and transferring a continuous stratum of said gelatin layer bearing said positive image, to an absorbent support.

3. The method of photographic reproduction which 45 comprises exposing to a subject a photographic element comprising a support having thereon an unhardened gelatino-silver halide emulsion layer and on said emulsion layer an unhardened gelatin layer having cadmium sulfide dispersed therein, developing said exposed emulsion layer with hydroquinone and N-methyl-p-aminophenol sulfate in the presence of sodium thiosulfate to 55 form a negative silver image in said emulsion layer and a positive nucleated silver image in said gelatin layer, and transferring a continuous stratum of said gelatin layer bearing said positive image, to an absorbent support.

#### References Cited in the file of this patent

#### UNITED STATES PATENTS

|              |        |               |
|--------------|--------|---------------|
| 2,500,421    | Land   | Mar. 14, 1950 |
| 2,543,181    | Land   | Feb. 27, 1951 |
| 2,565,377    | Land   | Aug. 21, 1951 |
| 70 2,596,754 | Yackel | May 13, 1952  |
| 2,647,056    | Land   | July 28, 1953 |

#### FOREIGN PATENTS

|    |        |             |               |
|----|--------|-------------|---------------|
| 75 | 59,365 | Netherlands | Apr. 17, 1947 |
|----|--------|-------------|---------------|